

March 21, 1933.

C. DANTSIZEN

1,902,493

WIRE MAKING PROCESS

Filed June 22, 1931



Fig. 2.

Iron Rod ~

Fig. 3.

Iron Rod ~  
Coating Comprising  
Ferric Hydrate  
and Lime

Fig. 4.

Iron Wire ~  
Coating Comprising  
Ferric Hydrate  
and Lime

Inventor:  
Christian Dantsizen,  
by Chabot & Cullar  
His Attorney.

## UNITED STATES PATENT OFFICE

CHRISTIAN DANTSIZEN, OF SCHENECTADY, NEW YORK, ASSIGNOR TO GENERAL ELECTRIC COMPANY, A CORPORATION OF NEW YORK

## WIRE MAKING PROCESS

Application filed June 22, 1931. Serial No. 548,169.

My invention relates to wire making processes and is concerned with a method of speeding up one of the ordinary processes of wire making generally used at present. The 5 invention is more particularly directed to that portion of the wire making process relating to the preparation of metallic rods for the wire drawing operation.

Generally speaking, the manufacture of 10 metallic wire, for example steel wire, according to one well known process comprises the fabrication first of wire rods by hot-rolling of the steel ingot and billet. These rods are usually hot-rolled to a diameter of about a 15 half inch or under and are subjected after suitable preparation to wire drawing operations to reduce them to the proper diameter.

One of the important steps in connection 20 with the making of wire is the proper preparation of the rods for the wire drawing operation. The rods must first be freed from scale or oxide else the die through which the wire is drawn will be ruined. The general practice is to remove the scale on the rods 25 with dilute sulphuric or hydrochloric acid.

After so cleaning the rods they are well washed and allowed to stand until they are 30 rusted (as termed by wire drawers, "browned") or in chemical terms they are coated with a film of ferric hydroxide. They may be kept under a spray of water until this brown rust forms. After the rod has rusted it is dipped into boiling lime water, drained and dried in ovens at about 100° C. The thin 35 coating of lime on top of the ferric hydrate serves the purpose of protecting the brown coat and also of keeping the rod from corroding and in addition acts as a dry lubricant in the subsequent wire drawing operations.

40 The rod is then subjected to drawing operations first through chilled iron dies and finally through steel and diamond dies.

This rusting and lime coating of the rod is exceedingly important and must be carried out with great care for the subsequent drawing operation depends very largely on the proper coating of the wire. At the present time there is a great loss of time and slowing down in the process of wire making being 45 cause of the fact that it takes anywhere from

a half hour to 24 hours to produce the requisite coat on the wire by allowing it to rust naturally in air. Since metal speeds down rapidly in the rolling mills from ingots to billets and rods preliminary to the drawing operations, it is the coating process now in vogue which holds up the process of finishing wire by drawing it through the dies.

I have discovered a method whereby I can materially speed up the process of putting on 60 the rust coat and lime on the rods prior to the drawing operations and hence materially speed up the entire process of wire making.

My process comprises briefly the making of 65 the rod anode for a few seconds in a bath of lime and water while passing current therethrough after which the rod is dried in air for a short period of time. In this manner I am able to quickly coat the rod with the proper rust coating and at the same time put 70 on the requisite coating of lime.

In the accompanying drawing forming 75 part of the present application Fig. 1 illustrates diagrammatically the process of the present invention.

Fig. 2 illustrates a cross section of the iron rod initially employed and before entering the lime bath.

Fig. 3 illustrates a cross section of the iron 80 rod after it has left the bath and been dried.

Fig. 4 illustrates a cross section of the iron wire after it has left the wire drawing dies.

In order to illustrate my invention but in no way limiting it the following example of 85 the process is given:

Iron rod 10 is rolled down to a suitable diameter, say,  $\frac{1}{4}$  inch and coiled if desired. It is then made the anode in a bath 11 of lime and water. Ordinarily a so-called solution of milk of lime is used as the bath. This is a saturated solution of calcium hydroxide carrying the excess of lime in suspension. Preferably an elevated temperature is employed. I have found a temperature of about 90° to 95 100° C. to be satisfactory. The time of treatment is very short, usually 5 to 15 seconds. A current density of 1 ampere per running inch of the rod is satisfactory. A separate cathode of any suitable material may be em- 100

ployed or the walls of the tank may be used as the cathode.

A gelatinous coating of ferrous hydrate is formed on the surface of the rod and this occurs and carries out of the bath with it an appreciable quantity of both free lime and its solution in water. On drying in air the green ferrous hydrate next to the rod rapidly oxides to brown ferric hydrate and probably 10 dehydrates partially to ferric oxide. The lime dries out also with the ferric hydrate. The rod is preferably fed continuously through the bath and at a rate such that it acquires the proper coating and is dried in 15 air after leaving the bath. Either air at room temperature or warmed air may be used. The coated rod, after leaving the bath and being dried, is fed through the usual wire drawing dies 12. The operation is thus 20 continuous. The separate coils of metallic rod may be made the anodes as such in the bath instead of being fed through the bath as outlined. It is preferred however to employ 25 the continuous process of coating and wire drawing.

It is thus apparent that by means of my discovery the entire process of wire making is materially speeded up. Not only is the 30 coating of the metal rod with ferric hydrate quickly accomplished, but also by means of my process the lime is deposited at the same time on the rod as the rust coat is being put on, thereby accomplishing in one operation 35 what it has heretofore been necessary to do in separate steps. Again by means of my invention a uniform coat of rust and lime is obtained and with proper control the coat may be made of any desired thickness.

As a result of my invention one practical 40 application is the production of welding wire for use in welding electrodes. It is known that a lime coating on an iron or steel electrode is a good weld-regulating substance. It is also known that such a coating adheres 45 with great tenacity and permanence if applied on or in conjunction with a sull or rust coating. As in the prior processes of making metallic wire the electrode rods have heretofore been allowed to rust naturally in air 50 after which they have been passed through a lime bath, dried and drawn through dies. There has been no control on the length of time required for putting the rust on the rods for this process, it will be appreciated, had to 55 vary with natural conditions. Nor was there any control of the amount of rust being put on. Great differences in performance of 60 welding wires probably are due to this lack of uniformity of coating on the wire. With the process of my invention the formation of the iron oxide coat is a matter of a few seconds instead of hours and the amount of iron oxide 65 produced as well as the amount of lime going on the wire is determined by the current density and the time of electrolysis.

What I claim as new and desire to secure by Letters Patent of the United States, is,—

1. The process of making wire which comprises fabricating a ferrous metallic rod of requisite thickness, making said rod the anode in a bath of lime and water, passing current therethrough, drying said rod, and drawing said rod through a wire drawing die.

2. The process of making wire which comprises fabricating a ferrous metallic rod of requisite thickness, making said rod the anode in a bath of lime and water for a few seconds while passing current therethrough and maintaining said bath at an elevated temperature, removing the rod from the bath, drying the rod in air, and drawing said rod through wire drawing dies to produce a wire of desired diameter.

3. The process of making wire which comprises fabricating a ferrous metallic rod of requisite thickness, making said rod the anode for about 5 to 15 seconds in a bath of lime and water maintained at a temperature of about 90-100° C. using a current density of approximately one ampere per square inch of rod surface, drying the rod in air, and passing it through a wire drawing die.

4. The process of making wire which comprises fabricating a ferrous metallic rod of requisite thickness, immersing said rod in a bath of lime and water, electrolytically depositing thereon a coating from said bath, removing said rod from said bath and drying it, and passing said rod through a wire drawing die.

5. The process of making wire which comprises fabricating a ferrous metallic rod of requisite thickness, passing said rod through a bath of lime and water, electrolytically depositing thereon a coating while said rod is passed through said bath, drying said rod after emergence from said bath, and passing said rod through a wire drawing die.

6. The process of making iron wire which comprises fabricating an iron rod of requisite thickness, continuously feeding said rod as anode through a bath of lime and water while passing current therethrough, the rate at which said rod is passed through said bath being sufficient to oxidize the surface thereof and deposit thereon a coating of lime from said bath, passing said rod from said bath into the air to dry said coating, and finally drawing the coated rod through a wire drawing die.

7. In the process of making wire the steps preliminary to the wire drawing operations which include making a ferrous metallic rod the anode in a bath of lime and water while passing current therethrough and subsequently drying the rod.

8. In the process of making wire the steps preliminary to the wire drawing operations which include making a ferrous metallic

rod the anode in a bath of lime and water for 5 to 15 seconds while passing current therethrough, the bath being maintained at an elevated temperature, and drying the rod

5 in air.

9. In the process of making wire the steps preliminary to the wire drawing operations which include producing a coating including ferric hydrate and lime on a ferrous metallic rod by making it the anode in a bath of lime and water, passing current therethrough, and drying the rod so treated in air.

10 In witness whereof, I have hereunto set  
15 my hand.

CHRISTIAN DANTSIZEN.